

## UNITED STATES PATENT OFFICE

2,491,238

## HEAT-TREATING IRON STEEL BODY

Lyman F. Whitney, Cambridge, Mass., assignor  
to Isthmian Metals, Inc., Boston, Mass., a cor-  
poration of Massachusetts

No Drawing. Original application August 16,  
1944, Serial No. 549,807. Divided and this ap-  
plication September 28, 1946, Serial No. 700,166

6 Claims. (Cl. 148—12)

1

This invention relates to the fabrication of articles made of iron or iron alloys, by pressing and sintering starting material which optionally has the final composition of the fabricated article. This starting material is in loose powder form.

An object of this invention is to produce a metal object of duplex structure such that one component consists of substantially carbon-free iron and another component consists of steel, one or both of these components being produced by powder metallurgy methods. A further object is to heat-treat objects of such duplex structure so that the steel component is hardened, while simultaneously the carbon-free iron component is softened or is unchanged in hardness.

Another object is to fabricate by powder metallurgy methods, a substantially carbon-free iron rotating band for steel artillery shells, the rotating band being attached to the shell either during fabrication of the band, or thereafter, and heat-treating the banded shell simultaneously to soften the iron band, and leave the shell in a hardened condition.

Many useful metal articles may consist of a duplex iron-steel structure. For example, artillery shells normally consist of a hard steel shell-body and a soft rotating band which, upon entering the gun barrel becomes sufficiently deformed to engage tightly the rifling of the barrel. The making of such rotating or shell bands from iron powder is one of the important uses for the method herein described.

In order to make an iron shell-band, the starting material may be a loose and freely-flowing iron powder.

This charge of loose iron powder is subjected to cold-pressing at a relatively light pressure of 15-40 tons per square inch.

This first cold-pressed body is sintered, without using pressure during the sintering, at 1600° F.-2000° F., during a sintering period of twenty minutes to one hour, and even up to three hours. As a specific example, the sintering temperature may be 1660° F., and the sintering period may be thirty minutes. As another specific example, the sintering temperature may be 1800° F. and the sintering period may be two hours.

This sintering is done in an inert or non-oxidizing atmosphere. For example, dry oxygen-free hydrogen or dry cracked oxygen-free ammonia gas provide a satisfactory sintering atmosphere for sintering an iron compact. When ammonia gas is cracked, nitrogen and hydrogen are produced. Dry and oxygen-free nitrogen and/or argon can also be used. If a cold-pressed steel

2

briquette or a mixture of iron and carbon is thus sintered, the atmosphere may be a dry and oxygen free mixture of hydrogen and methane or other stabilizing gas, intermixed in suitable proportion to prevent the sintering atmosphere from carburing or decarburing the briquette during the sintering. The sintered body should be cooled in the sintering atmosphere, until the sintered body will not oxidize when it is located in the air or in other oxidizing atmosphere. Hence, the sintered band is kept free from oxidation.

After the first sintering the compact is again cold pressed at a higher pressure to obtain the desired density. This higher pressure is preferably at least approximately 60 tons per square inch.

Normally a second sintering operation is useful after the second cold-pressing in order to eliminate or reduce the work-hardening which results from the second cold-pressing and in order to improve the physical properties of the body. The second sintering is performed under the same general conditions as the first sintering. The temperature of the second sintering can be 1500° F.-2000° F., the sintering period can be twenty minutes to one hour or more, and the sintered band is preferably allowed to cool slowly in the sintering atmosphere to 400° F.-500° F., as previously stated.

The upper limit of the sintering temperature may be as high as 2400° F., in sintering either iron or steel except that in sintering steel the sintering temperature should preferably be kept at least 100° F. below the melting point of the steel, which is being sintered. The melting point of the steel depends upon its carbon content.

Shell-bands made from said iron powder, according to the multiple-step method previously described, can be cold-swaged into the groove of the shell or other projectile, using the same method and apparatus which are now used for cold-swaging copper-alloy bands into said groove. This cold-swaging causes considerable work-hardening of the iron band, and it may be desirable to soften it by suitable heat-treatment. For example prior to the cold-swaging the iron band may have a hardness in the range Rockwell F 55-75, and after cold-swaging a hardness of Rockwell F 82-96. A typical steel shell-body has a hardness of Rockwell B 98-105. Such a shell-body containing a cold-swaged iron band can be heat-treated by heating it above the critical temperature of the steel (about 1400° F.) which is also above the recrystallizing temperature of the cold-worked iron band. This heating serves si-

multaneously to austenitize the steel and allow recrystallization and grain growth to take place in the iron. The banded shell may now be cooled at a carefully selected rate as hereinafter disclosed which will restore the steel to its original state of hardness, while the iron band will be found to have been softened to approximately its pre-swaging hardness. Alternatively, the banded shell may be quenched in water, brine, oil, or any other suitable medium. Such cooling will produce in the steel a high hardness, e. g. Rockwell C 40-60, but the iron band will not be hardened but rather will be restored to its preswaging hardness. The hardness of the steel shell may then be lowered to its original value by tempering.

*First alternative method*

As an alternative method of making a shell-band, the band can be annealed after it has been cold-swaged into the groove of the shell. In this alternative method, the iron powder may be cold-pressed in the manner previously mentioned, at a pressure of 10-60 tons per square inch to give bodies of substantially uniform densities of from 5.5 to 7.3. After sintering at 1800° F. under the conditions previously stated, such bodies may have a hardness of from 10 to 80 on the Rockwell H scale.

I can thus make said shell-band by a single cold-pressing and a single sintering, instead of using the four steps previously mentioned. This sintered iron band is cold-swaged to the groove of the shell-body. The work-hardening is then eliminated or reduced by annealing the banded shell-body at 1600° F.-1800° F., during an annealing period of two hours.

The higher annealing temperature of 1800° F. is preferred. The steel shell-body and its iron shell-band are then rapidly cooled from the annealing temperature, by a blast of non-oxidizing gas, to 20° C.-25° C. This cooling period may be 5-20 minutes. This rapid cooling converts the steel material of the shell-body from austenite, largely to pearlite, without substantially affecting the pure iron or ferrite of the iron band. This treatment removes or reduces the work-hardening of the iron band which has resulted from the cold-swaging.

Instead of using gas for said cooling, the banded shell-body can be quenched from above its critical temperature, in water or oil which is at a temperature of 20° C.-25° C. This critical temperature is about 1400° F., in an ordinary shell-body.

If the banded steel shell-body is thus quenched, the hardness of the banded steel shell-body is regulated by tempering or drawing in the well-known manner, by reheating the banded shell-body to a temperature below its critical range, so that the strength and hardness of the steel shell-body are brought to the proper value. Such tempering does not affect the hardness of the pure iron shell-band. In heat-treating the banded steel-body, the usual precautions are preferably taken to prevent oxidation of the iron band. In this method, the shell-body and its attached band are simultaneously and equally heat-treated. The hardness of the final annealed band is about 55-85 on the Rockwell F scale.

In a typical steel stock which is used for making a shell-body, the hardness of such steel stock is between 97.7-104.7 on the Rockwell B scale. The ultimate tensile strength of such steel stock is 99,700 lbs. per square inch to 128,800 lbs. per square inch.

In the finished shell-body with its completed band, the Rockwell B hardness of the steel stock is 96-104, after final heat treatment in the case in which the band and shell-body are heat treated after the band has been swaged on the shell-body.

The composition of a typical steel shell-body may be 0.30%-0.40% carbon, 1.15%-1.55% manganese, not more than 0.045% phosphorus, 0.075%-0.150% sulphur, and 0.15%-0.30% silicon, the remainder being iron.

*Second alternative method*

The loose iron powder is located in the groove of the shell-body, and the first cold-pressing is performed on said loose iron powder while it is so located, so that the first cold-pressed body is formed in situ in the groove. This cold-pressing can be done by using a die in which the shell-body is located. The pressure which is used in cold-pressing said loose and free-flowing iron powder in situ, may be 90 tons per square inch. The banded steel shell-body is then heated, as for example at 1600° F.-1800° F. during a heating period of two hours. The higher temperature of 1800° F. is preferred. Since this heat-treatment softens the steel body, its strength and hardness are adjusted by quenching and drawing, as in the first alternative method. A single pressing and a single heat-treatment are sufficient, in order to produce a satisfactory shell-band. A plurality of cold-pressing operations and sintering operations can be used.

As in the previous examples, the heat-treatment or sintering which succeeds the cold-pressing, eliminates or reduces the work-hardening which results from the cold-pressing, and improves the physical properties of the shell-band.

*Third alternative method*

It may also be desirable to make a duplex article which consists partly of relatively pure iron and partly of steel in which the steel component is made by powder metallurgy methods. In this case the powder metallurgy steel component can be hardened by heat treatment while the iron component is simultaneously softened or left unchanged in hardness. Such a heat treatment may consist of a heating at a temperature which is usually within the range 1400° F.-2000° F. followed by quenching in water or oil and subsequent tempering, or the cooling may be more slowly at a predetermined rate sufficient to result in the desired hardness of the steel component without subsequent tempering. During the heating it is preferable to surround the duplex body by protective atmosphere in order to prevent oxidation. If the heat treatment is relatively long (e. g. 15 minutes or over), it is preferable to use an inert atmosphere such as dry nitrogen or one of the noble gases. The more usual protective atmosphere such as partially burned gases, or cracked ammonia, or hydrogen, or mixtures of hydrogen and a hydrocarbon, may be suitable when the heating period is relatively short. However these atmospheres react on iron or steel and during a prolonged heat treatment may either carburize the iron or decarburize the steel or both since it is impossible for such atmosphere to be simultaneously in equilibrium with iron and steel.

In order to produce by powder metallurgy methods steel compacts suitable for hardening by conventional heat treatments the following procedure may be used.

According to one method which is within the scope of my invention, the iron powder is mixed with the proper proportion of graphite, a briquette is made of this mixture by cold-pressing at 15-40 tons per square inch, and this briquette is then heated and thus sintered in an atmosphere which prevents any injurious loss of the graphite during the sintering operation. Preferably this sintering operation is carried out at a temperature of 2000° F. and for a period of from one to three hours, in an atmosphere of methane and hydrogen.

The methane can be replaced by propane or other stabilizing gas.

It is desired to combine all the graphite with the iron powder. Hence the proportion of graphite is the desired final proportion of combined carbon in the final steel body. The proportion of methane in the sintering atmosphere depends upon the sintering temperature and the final proportion of combined carbon which it is desired to have in the final steel product. The methane acts as a stabilizing gas, so that the graphite combines with the iron, and not with the hydrogen. The proportion of methane must not be excessive, or else some of the methane will be decomposed, and the resultant liberated carbon will combine with the iron, to over-carburize the steel beyond the desired limit. Hence the proportion of methane is selected so that the briquette neither loses nor gains carbon during the sintering, and the proportion of combined carbon in the final steel material is determined by the proportion of graphite in the briquette.

As elsewhere explained herein, it is very important to provide a sintering atmosphere during carburization, which is free from water vapor and oxygen. Hence the commercial hydrogen and stabilizing gas mixture is purified by removing the oxygen, and water vapor is also removed, as further explained herein.

After the first sintering when the iron has combined with the graphite the briquette is again cold pressed at a higher pressure to obtain the desired density and then resintered. This higher pressure is preferably at least approximately 60 tons per square inch.

Steel compacts made as described above may be combined with iron bodies made from wrought material or by powder metallurgy methods by any of several methods for example the two may be joined by copper brazing, swaging, by riveting etc. Alternatively they may be joined during the powder metallurgy operations of pressing and sintering.

This application is a division of copending application Ser. No. 549,807, filed August 16, 1944, now Patent No. 2,411,073, for Making products of iron or iron alloys.

I claim:

1. A method of making a duplex metal body of ferrous metal parts of different hardenability and wherein the separate or assembled parts in their ultimate shape cannot be assembled or disassembled, comprising the steps of preforming one part to its ultimate dimensions, preforming the other part to such dimensions as will permit its assembly with the one part, assembling the parts, deforming the said other part into intimate mechanical engagement with said one part, said deformation of said other part being accompanied by severe internal work hardening, and then withdrawing the work hardening from said deformed other part by heat treating the duplex

body at a temperature which is above the recrystallization temperature of the deformed part.

2. A method of making a duplex metal body of iron and steel parts wherein the steel part is relatively harder than the iron part and wherein the separate or assembled parts in their ultimate shape cannot be assembled or disassembled, comprising the steps of preforming the steel part to its ultimate dimensions, preforming the soft iron part to such dimensions as will permit its assembly with the steel part, assembling the parts, deforming the iron part into intimate mechanical engagement with the steel part, said deformation of the iron part being accompanied by severe internal work hardening, and then withdrawing the work hardening from the deformed iron part by heat treating the duplex body at a temperature which is above the recrystallization temperature of the deformed iron part.

3. The method of making a duplex metal body of interengageable preformed iron and steel parts of different hardenability, the ultimate shape of the parts being such that prior to assembly at least one part must have dimensions different from its final dimensions to permit interengagement of said part with said other part, and that following assembly and deformation to interengage the parts they cannot be disassembled without destruction of one of the parts, comprising the steps of preforming the steel part to its ultimate shape, preforming the iron part to such dimensions as will permit assembling it with the steel part, assembling the parts, deforming the iron part into intimate mechanical engagement with the steel part, said deformation of the iron part being accompanied by severe internal work hardening, and then withdrawing the work hardening from the iron part by heat treating the duplex body at a temperature which is above the recrystallization temperature of the deformed iron part.

4. A method of making a duplex metal body of iron and steel parts wherein the steel part is relatively harder than the iron part and wherein the separate or assembled parts in their ultimate shape cannot be assembled or disassembled, comprising the steps of preforming the steel part to its ultimate dimensions, preforming the soft powder iron part to such dimensions as will permit its assembly with the steel part, assembling the parts, deforming the soft iron part into intimate mechanical engagement with the steel part, said deformation of the iron part being accompanied by severe internal work hardening, and then withdrawing the work hardening from the deformed iron part by heat treating the duplex body at a temperature which is above the recrystallization temperature of the deformed iron part without changing the hardness of the steel part.

5. A method of making a duplex metal body of iron and steel parts wherein the steel part is relatively harder than the iron part and wherein the separate or assembled parts in their ultimate shape cannot be assembled or disassembled, comprising the steps of preforming the steel part to its ultimate dimensions, preforming the soft powder iron part to such dimensions as will permit its assembly with the steel part, assembling the parts, deforming the soft iron part into intimate mechanical engagement with the steel part, said deformation of the iron part being accompanied by severe internal work hardening, and then withdrawing the work hardening from the deformed iron part by heat treating the duplex

plex body at a temperature which is above the recrystallization temperature of the deformed iron part and concomitantly increasing the hardness of the steel part.

6. A method of making a duplex metal body of iron and steel parts wherein the steel part is relatively harder than the iron part and wherein the separate or assembled parts in their ultimate shape cannot be assembled or disassembled, comprising the steps of preforming the steel part to its ultimate dimensions, preforming the soft powder iron part to such dimensions as will permit its assembly with the steel part, assembling the parts, deforming the soft iron part into intimate mechanical engagement with the steel part, said deformation of the iron part being accompanied by severe internal work hardening, and then withdrawing the work hardening from the deformed iron part by heat treating the du-

5

plex body at a temperature which is above the recrystallization temperature of the deformed iron part and concomitantly decreasing the hardness of the steel part.

10

LYMAN F. WHITNEY.

## REFERENCES CITED

The following references are of record in the file of this patent:

## UNITED STATES PATENTS

| Number    | Name             | Date          |
|-----------|------------------|---------------|
| 2,209,709 | Weatherhead, Jr. | July 30, 1940 |
| 2,275,420 | Clark et al.     | Mar. 10, 1942 |

## FOREIGN PATENTS

| Number  | Country       | Date          |
|---------|---------------|---------------|
| 398,045 | Great Britain | Sept. 7, 1933 |